

## UNITED STATES PATENT OFFICE

ELMER M. JONES, OF DETROIT, MICHIGAN, ASSIGNOR TO PARKER RUST-PROOF COMPANY, OF DETROIT, MICHIGAN, A CORPORATION OF MICHIGAN

## COATED IRON AND STEEL ARTICLES AND METHOD OF MAKING THE SAME

No Drawing.

Application filed June 13, 1927. Serial No. 198,696.

This invention relates to coated iron and steel articles, and a method of producing the desired coating on the articles.

More specifically, the invention relates to iron or steel articles provided with a coating containing a compound of silicon, and to a method of providing such a coating.

The coating to which the invention relates may be relied upon to protect the surfaces to 10 which it is applied, or it may be used as a foundation for another coating.

One important advantage of the invention is that the coating to which it relates may be applied to pickled surfaces of iron or steel 15 without intermediate preparatory operations other than washing.

One specific method of providing iron or steel surfaces with a coating formed in situ, and containing a compound of silicon, will 20 be described with sufficient detail to enable those skilled in the art to carry out the method, and thereafter some modifications of the described method will be discussed.

A dilute solution of phosphoric acid is 25 formed, and a compound of silicon is introduced into this solution. The solution may be formed by dissolving in water acid phosphates of iron, manganese or zinc, or a combination of the acid phosphates of two or 30 more of these metals, formed as described in a co-pending application of applicant with Hobart H. Willard and Matthew Green, Ser. No. 83,736, filed Jan. 25, 1926, which eventuated into Patent No. 1,651,694 December 6, 35 1927, and preferred proportion is about twenty pounds of the phosphates to 125 gallons of water. The silicon compound may be ordinary sand.

This solution is boiled, and after four or 40 five hours of boiling there is produced a whitish colloidal material which is apparently silicic acid.

After the appearance of the silicic acid, articles having surfaces of iron or steel are 45 placed in the boiling solution, and a coating immediately begins to form on said surfaces. The exact chemical formulas of the ingredients of this coating have not been determined, but the coating is known to comprise 50 insoluble phosphates of the metals whose sol-

uble acid phosphates were introduced into the bath, and a silicon compound which is apparently a silicate of iron.

The silicic acid must be brought into contact with the surfaces to be coated in order 55 to produce the silicon compound in the coating. The colloidal silicic acid is so nearly the specific gravity of water that it is readily distributed throughout the bath by slight agitation. For a small tank, merely boiling produces sufficient agitation to distribute the silicic acid; but when boiling is not sufficient to bring the silicic acid into contact with the surfaces to be coated, other agitating means may 60 be employed.

The coating readily forms on any clean 65 surface of iron or steel, including a pickled surface. It is preferable to wash the articles to be coated after pickling, in order to avoid useless waste of chemicals in the coating bath, 70 but other preparatory treatment of pickled surfaces is unnecessary.

If desired, the articles may be left in the 75 bath for an hour or so, or until the formation of coating ceases. Hydrogen is given off during the formation of the coating, so that the completion of the coating operation is indicated by the cessation of the hydrogen bubbles. If the coating operation is carried to this limit, the resultant coating is sufficiently 80 thick to provide an efficient protection against rusting.

If an external coating of a different nature 85 is desired, the described coating may be used as a foundation, whether the operation is carried to its limit or is stopped far short of that limit. The coating is formed in situ and is integral with, or very intimately associated with, the coated article, and is very evenly distributed over the surface, so that it forms 90 a very good foundation coating. As brief a period as five minutes suffices to produce a coating sufficient to furnish a foundation for subsequent coating operations.

A well known process of rust-proofing iron 95 and steel surfaces has been to subject such surfaces to boiling in a dilute solution of phosphates of iron, manganese, zinc, etc. One difficulty encountered in carrying out this process is that articles cleaned by pickling 100

cannot be successfully rust-proofed by this method without intermediate treatment. With untreated pickled articles the bath containing phosphates of iron either does not attack the work at all, or produces a coating having large crystals at separated intervals in a comparatively thin and ineffective coating. This produces what has been known in the trade as "sparkle", recognized by the sparkling of the large crystals, and unsatisfactory as a rust-proofing coating.

Various methods of treating the surfaces after pickling in order to prepare them for rust-proofing have been employed. Rubbing or brushing the surfaces, particularly tumbling the articles in sand, is effective to prepare the surfaces for receiving a satisfactory coating, but there are many articles which are not adapted for such tumbling in sand, and individual brushing or treatment of the articles is necessarily troublesome and expensive.

Where it is desired to apply the customary coating of phosphates of iron, or similar phosphates, the articles may be dipped for a short time in the bath first described, after having been pickled and washed, and then transferred to the usual rust-proofing tank. This preliminary treatment in the bath containing silicic acid results in a much quicker operation in the regular rust-proofing tank, as well as eliminating the difficulty described above as "sparkle".

Difficulty is encountered in providing pickled surfaces of iron or steel with other coatings, such as enamel or pyroxylin finish or ordinary paint, for example, without intermediate treatment of the surfaces after pickling. A preparatory coating formed in the bath of dilute phosphoric acid containing colloidal silicic acid forms a good foundation for such other coatings as well as for further coating with phosphates.

Ordinary sand is referred to above, but other materials containing silica may be used to produce the necessary silicic acid. The preliminary boiling necessary to bring the bath to proper condition for coating may be shortened by the use of fused silica, or silica in other forms that are more readily attacked by the acid in the solution.

One way in which the bath containing phosphates may be formed has been described, but it will be readily understood that a similar bath may be formed in other ways. The silicic acid may be produced in other ways either in the bath or separately and introduced into the bath; and the dilute solution of phosphoric acid and phosphates may be produced in any of the known ways for producing such a rust-proofing solution. However, after the bath is once formed, the introduction of sand into the bath to maintain the supply of silicic acid is simple and effective, as sufficient silicic acid is formed

during the regular coating process to maintain a supply, and nothing further than the presence of the sand in the bath during the coating operation is necessary to maintain the necessary silicon compounds in the bath. 70

The phosphoric acid or acid phosphate content of the bath may be maintained in any of the known ways for maintaining such a solution, but the method at present preferred is the use of the powder formed in accordance with the disclosure of the patent identified above. 75

Where a dilute solution of phosphoric acid is referred to in the appended claims, it will be understood that a solution is referred to 80 which is suitable for coating surfaces of iron or steel with insoluble phosphates.

Having described the nature of my invention and a method of carrying it out, what I claim is:

1. Iron or steel articles, or articles having surfaces of iron or steel, having a coating formed in situ on said surfaces and comprising a silicate of iron and a phosphate. 85

2. Iron or steel articles, or articles having surfaces of iron or steel, having a coating formed in situ on said surfaces and comprising insoluble phosphates of metals and a compound of silicon. 90

3. The method of coating an article having a surface of iron or steel roughened as by pickling, which comprises bringing into contact with said surface a colloidal material capable of reacting with phosphates to form an insoluble material, and subjecting said material to the action of phosphates while in contact with said surface. 95

4. The method of providing an article having a surface of iron or steel with a coating which consists in boiling said article in a dilute solution of phosphoric acid containing colloidal silicic acid. 100

5. The method of coating pickled surfaces of iron or steel, which consists in boiling articles having such surfaces in a dilute solution of phosphoric acid containing colloidal silicic acid. 105

6. The method of coating articles having surfaces of iron or steel, which consists in forming a dilute solution of phosphoric acid containing a compound of silicon, boiling the solution until colloidal silicic acid is formed, and thereafter subjecting said surfaces to the action of the boiling solution. 110

7. A method of preparing for coating articles having surfaces of iron or steel, which consists in pickling said surfaces, thereafter washing the surfaces and applying to the surfaces a boiling dilute solution of phosphoric acid containing colloidal silicic acid 115 for a sufficient time to form a foundation film over said surfaces. 120

8. A bath for coating articles having surfaces of iron or steel roughened as by pickling, comprising a dilute solution containing 125

phosphoric acid radical and a colloidal material capable of reacting with said radical to form an insoluble product.

9. A bath for coating articles having surfaces of iron or steel, comprising a dilute solution of phosphoric acid containing colloidal silicic acid.

In testimony whereof, I have hereunto signed my name to this specification.

10 ELMER M. JONES.

15

20

25

30

35

40

45

50

55

60